

R. SINCLAIRE.

FLYING TARGET.

APPLICATION FILED JUNE 28, 1915.

1,203,147.

Patented Oct. 31, 1916.

Fig. 1.



Fig. 2.



Fig. 3.



Inventor  
*R. Sinclair*

By  
*Verne M. Koseny*

Attorney.

# UNITED STATES PATENT OFFICE.

REGINALD SINCLAIRE, OF CORNING, NEW YORK.

## FLYING TARGET.

1,203,147.

Specification of Letters Patent. Patented Oct. 31, 1916.

Application filed June 28, 1915. Serial No. 36,763.

*To all whom it may concern:*

Be it known that I, REGINALD SINCLAIRE, a citizen of the United States of America, and a resident of Corning, New York, have 5 invented certain new and useful Improvements in Flying Targets, of which the following is a specification.

Flying targets of to-day are generally made of a clay cemented together with a 10 bituminous cement, and are commonly known as clay-pigeons. Such pigeons, while essentially fragile in transportation, and liable to break when falling to the ground unhit by shot, are not sufficiently sensitive 15 to the impact of the shot to insure their breaking when hit by only one or a few pellets. Inasmuch as it is the practice to count as "hits" only the "pigeons" actually shattered into pieces by the impact of a shot, 20 and as pigeons broken on falling to the ground are destroyed for future use, the importance of increasing the percentage of breaks when the pigeons are struck and reducing the percentage of breaks resulting 25 from unstruck pigeons falling upon the ground will be appreciated. The present clay pigeon is a compromise in this respect, the percentage of "breaks" from shot impact and "recoveries" from pigeons picked 30 up, being balanced against each other.

It is the object of this invention to provide a pigeon which will have a greatly increased percentage of breaks, without a decrease of the percentage of recoveries, and 35 indeed in the embodiment here shown with a higher increased percentage of recoveries.

For these purposes, the invention consists in a target a part at least of which is under internal tensile stress, so that any crack 40 created by the impact of the shot, is by the internal stresses of the target, developed into a complete disintegration and breaking up thereof.

In the preferred embodiment here shown, 45 the target is of the form in which clay pigeons are commonly made, that is to say of a more or less concaved disk, the outer and upper surface of which is held under initial tensile strain by the inner and lower surface, and the material used in the construction of this preferred embodiment is glass or a vitreous composition of the same general character.

Referring to the accompanying drawings, 50 in which corresponding parts are designated

by similar marks of reference,—Figure 1 is a face view of a pigeon or target made in accordance with this invention. Fig. 2 is a cross section thereof. Fig. 3 illustrates a suitable press mechanism for forming a target 60 in accordance with this invention.

Referring to Fig. 1, it will be seen that the target is of the shape and contour now commonly employed with the clay pigeon, that is to say, it is a concaved disk embodying a central dome 1, and an outer flange 2 connected to the central dome by the inclined petticoat 3. In the embodiment shown, this target is made of glass, preferably by pressing in a mold in the ordinary 70 manner as is shown in Fig. 3. This mold as usual, consists of the mold-proper 4, and the plunger 5, the plunger being adapted to form the inner concaved side of the pigeon. If glass is the material employed, and the 75 mold plunger be properly cooled, (it being shown for this purpose as hollow to permit water circulation therein), the glass 10 in contact with and adjacent to such plunger will be quickly set, while the outer convex 80 upper surface 11 of the pigeon will be more slowly set by the hotter mold. Under these conditions, internal stresses will be set up in the glass, and the outer surface be under tension, and thus ready to disintegrate and go 85 to pieces upon a slight fracture. By experiments, it has been found that targets made in this manner are fractured in a larger proportion of cases than ordinary clay pigeon, by the impact of a single shot. 90

It will be seen that not only can the stress left in the pigeon be regulated by the stress initially placed within it due to the relative temperature of the mold and plunger, but that also such stress, after being initially 95 placed therein may be reduced by proper annealing to insure greater chance of recovery. In practice, this stress will be so adjusted as to insure breaking upon impact of shot in a high percentage of cases, and 100 also to permit recovery when unhit. I have found that a glass pigeon, even with the internal stresses necessary to insure breaking by the single shot, has sufficient mechanical strength to prevent it breaking when 105 falling on the ordinary shooting ground.

It is obviously possible instead of forming a pigeon in one operation as here shown, to form it in two operations, that is to say, to form the inner part of the pigeon in one 110

pressing, and to cast around it a layer of glass of the same or of different co-efficient of expansion, or to form the pigeon in the same pressing operation of two glasses having different co-efficient of thermal expansion. Likewise, my invention is not restricted to forming the pigeon of the material here shown, to-wit, glass, for the stresses here described may be produced with other fragile material as for instance, by using two plates of different expansion co-efficient of drying shrinkages, or by using a clay or other fragile material, and more rapidly drying or setting of one of the sides.

Having thus described my invention what I claim is:

1. A flying target consisting of an integral disk of a frangible material, such disk being under internal tensile strain.
2. A flying target consisting of a concaved integral disk, the exterior of such disk being

held under internal tensile strain by the interior of such disk.

3. An integral flying target consisting of a central dome, and a surrounding flange connected to the dome by a petticoat, the outer surface of the target being held under internal tensile strain by the inner surface thereof.

4. An integral flying target consisting of frangible material having its outer surface under tensile strain.

5. An integral flying target of glass having its outer surface under initial tensile strain.

In testimony whereof I have signed my name in the presence of two witnesses.

REGINALD SINCLAIRE.

Witnesses:

J. T. LITTLETON, Jr.,  
W.M. C. TAYLOR.

Copies of this patent may be obtained for five cents each, by addressing the "Commissioner of Patents, Washington, D. C."